

Feb. 20, 1962

A. OSSENBRUNNER ETAL

3,022,171

PHOTOGRAPHIC FILTER AND ANTIHALATION LAYERS

Filed July 16, 1957



ARMIN OSSENBRUNNER, HELFRIED KLOCKGETHER,

INVENTORS

BY

*Connolly and Hutz*  
THEIR ATTORNEYS.

# United States Patent Office

3,022,171

Patented Feb. 20, 1962

1

3,022,171

## PHOTOGRAPHIC FILTER AND ANTIHALATION LAYERS

Armin Ossenbrunner and Helfried Klockgether, Leverkusen, Germany, assignors to Agfa Aktiengesellschaft  
Filed July 16, 1957, Ser. No. 672,199  
Claims priority, application Germany July 26, 1956  
16 Claims. (Cl. 96—84)

The present invention relates to light-absorbing photographic layers and more particularly to antihalation and filter layers for light sensitive photographic materials comprising silver halide emulsion layers.

It is known to provide photographic materials, such as black-and-white films and multi-layer color films, with an antihalation layer so as to avoid the formation of halation. This antihalation layer is arranged either between layers or on the back of the support. The antihalation layer generally consists of an antihalation dye which is removed in the photographic processing baths, and a binding agent, generally gelatine or, because of their better mechanical properties, alkali-soluble plastics.

The following are known examples of such plastics:

Copolymers of styrene and acrylic acid, vinyl isobutyl ether and maleic acid, vinyl butyl ether and maleic acid, and styrene and maleic acid, according to U.S. patent specification No. 2,077,789;

Condensation products of phenoxyacetic acid and formaldehyde, according to U.S. patent specifications Nos. 2,075,145; 2,089,764 and 2,282,890;

Copolymers of acrylonitrile, vinyl butyl ether and maleic acid semi-esters, according to U.S. application Serial No. 622,088, filed November 14, 1956, now U.S. Patent 2,913,351, granted November 17, 1959 (Belgian Patent No. 552,893);

Cellulose acetate phthalates, polyvinyl phthalates according to U.S. patent specification No. 2,131,747.

In actual fact, however, the standards required of an antihalation layer are so high that only a few of the aforementioned binding agents can be considered for practical use in the manufacturing processes. In addition, recent research has developed entirely new types of materials for the support for which the existing dye carriers are not always the best possible. When a suitable synthetic resin is chosen as a binding agent for the antihalation layer the following requirements should be fulfilled:

(1) Sufficient solubility in organic solvents which are at the same time solvents for the antihalation dye, and which should cause no or only slight swelling of the layer support, since if swelling does occur the support becomes colored.

(2) Sufficient solubility in the developers, which are often only weakly alkaline, so that no residues remain after processing.

(3) The smallest possible tendency to transfer to the emulsion layer disposed in contact with the antihalation layer. Any such transfer makes the film material unsuitable for use.

It is these last two requirements which are difficult to fulfill. An increase in the groups in the molecule which produce alkali solubility improves the solubility in the alkaline developers, but reduces the resistance to transfer due to the resulting more hydrophilic properties, while on the other hand a reduction in the groups producing alkali solubility improves the resistance to transfer, but reduces the solubility in the photographic baths.

It has now been found that antihalation layers can be produced which have excellent properties if high molecular alkali-soluble polycarbonic acid esters of aliphatic, cycloaliphatic, araliphatic and/or aromatic dihydroxy compounds containing acid groups, optionally in admix-

2

ture with organic dihydroxy compounds without acid groups are used as binding agents. These polycarbonic acid esters contain recurring units of the formula:



in which R stands for a bivalent organic radical containing as sole reactive group an acid group, such as at least one carboxylic and/or sulphonic acid group, whereby in

10 part of these recurring units R may stand for a bivalent organic radical containing no acid groups or other reactive groups, said bivalent organic radical being derived from the aforementioned organic dihydroxy compounds by subtraction of the hydroxy groups. In case part of 15 said recurring units contain no acid groups, these are present in such molar proportion that the polycarbonate does not lose its solubility in aqueous alkaline solution, these molar proportions being about 1-70 molar percent as calculated on the total molar weight of recurring units. 20 As represented in the above formula these polycarbonic acid esters are linear.

The alkali-soluble polycarbonic acid esters of high molecular weight which are to be used in accordance with the invention can be obtained by reacting aliphatic, cyclo-

25 aliphatic, araliphatic or aromatic dihydroxy compounds containing acid groups, if desired admixed with cycloaliphatic, araliphatic or aromatic dihydroxy compounds without acid groups, with carbonic acid chlorides such as bis-halogen carbonic acid esters of dihydroxy compounds

30 or with phosgene, for example according to the prescription given in German application F-13,040 (now German Patent 971,790) or Belgian Patent 532,543. Such polycarbonates can thus contain the radicals of dihydroxy carboxylic acids such as tartaric acid, dihydroxy stearic acids, 2,5-dihydroxycyclohexane carboxylic acid, 4,4'-di-

35 hydroxydicyclohexyl carboxylic acid-(2,2'), 1,5-dihydroxy benzoic acid, 3,6-dihydroxybenzene-1,2-dicarboxylic acid, 4,4'-dihydroxydiphenyl-2,2'-dicarboxylic acid and especially di-(monohydroxy aryl)alkanes containing carboxyl

40 groups, such as 4,4'-dihydroxy-3,3'-dicarboxy diphenylmethane and 4,4'-dihydroxy-3,3'-dicarboxy-5,5'-dimethyl diphenyl methane, and also dihydroxysulphonic acids such as 1,4-dihydroxybenzene sulphonic acid-(2), 1,6-dihydroxynaphthalene sulphonic acid-(3) and 4,4'-dihydroxy diphenyl disulphonic acid-(2,2'), or 2,2[4,4'-dihydroxy-diphenylene - disulphonic acid - (3,3')] - propane. Particularly suitable for the process of the invention are those polycarbonic acid esters, for the production of which 4,4'-dihydroxy-3,3'-dicarboxy diphenyl methane or 4,4'-dihydroxy - 3,3' - dicarboxy - 5,5' - dimethyl diphenyl methane have been used.

Other dihydroxy compounds which in addition may be used, if desired, for the production of the polycarbonates are:

55 As aliphatic dihydroxy compounds—ethylene glycol, diethylene glycol, triethylene glycol, polyethylene glycol, thiodiglycol, ethylene dithiodiglycol, the di- and polyglycols produced from propyleneoxide-1,2, o, m, or p-xylene glycol, propanediol-1,3, butanediol-1,3, butanediol-1,4, 2-methylpropanediol-1,3, pentanediol-1,5, 2-ethylpropanediol-1,3, hexanediol-1,6, octanediol-1,8, 1-ethylhexanediol-1,3, and decanediol-1,10,

60 As cycloaliphatic dihydroxy compounds—cyclohexane-diol-1,4, cyclohexanediol-1,2, 2,2-(4,4'-dihydroxy-dicyclohexylene)-propane and 2,6-dihydroxydecahydronaphthalene,

65 As aromatic dihydroxy compounds—hydroquinone, resorcinol, pyrocatechol, 4,4'-dihydroxydiphenyl, 2,2-dihydroxydiphenyl, 1,4-dihydroxynaphthalene, 1,6-dihydroxynaphthalene, 2,6-dihydroxynaphthalene, 1,2-dihydroxynaphthalene, 1,5-dihydroxynaphthalene, dihydroxyanthra-

## 3

cene, 2,2-dihydroxydinaphthyl-1,1' and o, m, p-hydroxybenzylalcohol.

Preferred classes of aromatic dihydroxy compounds are the di-monohydroxy arylene sulphones and particularly the di-monohydroxy arylene alkanes, such as 4,4'-dihydroxy-diphenylene sulphone, 2,2'-dihydroxydiphenylene sulphone, 3,3'-dihydroxydiphenylene sulphone, 4,4'-dihydroxy-2,2'-dimethyl-diphenylene sulphone, 4,4'-dihydroxy-3,3'-dimethyl-diphenylene sulphone, 2,2'-dihydroxy-4,4'-dimethyl-diphenylene sulphone, 4,4'-dihydroxy-2,2'-diethyl-diphenylene sulphone, 4,4'-dihydroxy-3,3'-diethyl-diphenylene sulphone, 4,4'-dihydroxy-2,2'-di-tert.butyl-diphenylene sulphone, 4,4'-dihydroxy-3,3'-di-tert.butyl-diphenylene sulphone and 2,2'-dihydroxy-1,1'-dinaphthylene sulphone, 4,4'-dihydroxy-diphenylene-methane,

10 15

1,1-(4,4'-dihydroxy-diphenylene)-ethane,  
1,1-(4,4'-dihydroxy-diphenylene)-propane,  
1,1-(4,4'-dihydroxy-diphenylene)-butane,  
1,1-(4,4'-dihydroxy-diphenylene)-2-methyl-propane,  
1,1-(4,4'-dihydroxy-diphenylene)-heptane,  
1,1-(4,4'-dihydroxy-diphenylene)-1-phenyl-methane,  
1,1-(4,4'-dihydroxy-diphenylene)-(4 - methyl - phenylene)-methane,  
(4,4' - dihydroxy - diphenylene) - (4 - ethyl - phenylene)-methane,  
(4,4' - dihydroxy - diphenylene) - (4 - isopropyl - phenylene)-methane,  
(4,4' - dihydroxy - diphenylene) - (4 - butyl - phenylene)-methane,  
(4,4' - dihydroxy - diphenylene)-benzyl-methane,  
(4,4' - dihydroxy - diphenylene)- $\alpha$ -furyl-methane,  
2,2-(4,4'-dihydroxy-diphenylene)-propane,  
2,2-(4,4'-dihydroxy-diphenylene)-butane,  
2,2-(4,4'-dihydroxy-diphenylene)-pentane (melting point 149-150° C.),  
2,2-(4,4'-dihydroxy-diphenylene)-4-methyl-pentane,  
2,2-(4,4'-dihydroxy-diphenylene)-heptane (boiling point 198-200° C. under 9.3 mms. mercury gauge),  
2,2-(4,4'-dihydroxy-diphenylene)-octane,  
2,2-(4,4'-dihydroxy-diphenylene)-nonane (melting point 68° C.),  
1,1-(4,4'-dihydroxy-diphenylene)-1-phenyl-ethane,  
(4,4'-dihydroxy-diphenylene)-1-( $\alpha$ -furyl)-ethane,  
3,3-(4,4'-dihydroxy-diphenylene)-pentane,  
4,4-(4,4'-dihydroxy-diphenylene)-heptane,  
1,1-(4,4'-dihydroxy-diphenylene)-cyclopentane,  
1,1-(4,4'-dihydroxy-diphenylene)-cyclohexane,  
2,2 - (4,4'-dihydroxy-diphenylene)-decahydronaphthalene (melting point 181° C.),  
2,2-(4,4' - dihydroxy - 3,3' - dicyclohexyl - diphenylene)-propane (melting point 144-146° C.),  
2,2-(4,4'-dihydroxy - 3 - methyl - diphenylene)-propane (melting point 114° C.),  
2,2-(5,5'-dihydroxy-3-isopropyl-diphenylene)-butane,  
1,1-(4,4'-dihydroxy - 3,3' - dimethyl-diphenylene)-cyclohexane,  
2,2-(4,4'-dihydroxy-3,3'-butyl-diphenylene)-propane,  
2,2-(4,4'-dihydroxy-3,3'-diphenyl-diphenylene)-propane,  
2,2-(4,4'-dihydroxy-2,2'-dimethyl-diphenylene)-propane,  
1,1 - (4,4'-dihydroxy-3,3'-dimethyl-6,6'-dibutyl-diphenylene)-butane,  
1,1 - (4,4'-dihydroxy-3,3'-dimethyl - 6,6' - di-tert.butyl-diphenylene)-ethane,  
1,1-(4,4'-dihydroxy - 3,3' - dimethyl-6,6'-di-tert.butyl-diphenylene)-propane,  
1,1 - (4,4' - dihydroxy - 3,3' - dimethyl-6,6'-di-tert.butyl-diphenylene)-butane,  
1,1 - (4,4' - dihydroxy - 3,3' - dimethyl-6,6'-di-tert.butyl-diphenylene)-isobutane,  
1,1 - (4,4'-dihydroxy-3,3'-dimethyl - 6,6' - di - tert.butyl-diphenylene)-heptane,  
1,1 - (4,4'-dihydroxy - 3,3' - dimethyl - 6,6' - di-tert.butyl-diphenylene)-1-phenyl-methane,

20 25

30 35

40

45 50

55 60

65 70

70

1,1 - (4,4' - dihydroxy - 3,3' - dimethyl-6,6'-di-tert.butyl-diphenylene)-2-methyl-pentane,  
1,1 - (4,4' - dihydroxy - 3,3' - dimethyl-6,6'-di-tert.butyl-diphenylene)-2-ethyl-hexane, and  
1,1 - (4,4' - dihydroxy - 3,3' - dimethyl-6,6'-di-tert.amyl-diphenylene)-butane,  
2,2-(4,4'-dihydroxy-dinaphthylene)-propane and  
1,1-(4,4'-dihydroxy-dinaphthylene)-cyclohexane.

Among the great number of suitable di-monohydroxy arylene alkanes the 4,4'-dihydroxy-diphenylene alkanes are preferred, especially the 2,2-(4,4'-dihydroxy-diphenylene)-propane and the 1,1 - (4,4' - dihydroxy-diphenylene)-cyclohexane.

The polycarbonates can be produced for example by introducing phosgene into solutions of dihydroxy compounds or of mixtures of the aforesaid dihydroxy compounds in organic bases, such as dimethylaniline, diethyl-aniline, trimethylamine, and pyridine, or in indifferent organic solvents, such as petrol, ligroin, cyclohexane, methylcyclohexane, benzene, toluene, xylene, chloroform, methylenechloride, carbon tetrachloride, trichloroethylene, dichloroethane, methacetate, and ethylacetate, with addition of an acid-binding agent, e.g. tertiary amines.

A process particularly suitable for producing polycarbonates consists in introducing phosgene into the aqueous solution or suspension of alkali or alkaline earth metal salts, such as lithium, sodium, potassium, and calcium salts of the dihydroxy compounds, preferably in the presence of an excess of a base, such as lithium, sodium, potassium, and calcium hydroxide or carbonate. The polycarbonate then precipitates out from the aqueous solution.

The conversion in the aqueous solution is promoted by the addition of solvents of the kind mentioned above which are inert to the reaction and capable of dissolving phosgene and eventually the produced polycarbonate.

The reaction conditions should preferably be so that one mole of the phosgene reacts with one mole of the dihydroxy compounds. Suitable temperatures are from about 0° C. to 100° C.

It is also possible to react the dihydroxy compounds containing acid groups, if desired in admixture with other dihydroxy compounds, with bis chlorocarbonic acid esters of dihydroxy compounds such as glycol-bis-chlorocarbonic acid ester, butanediol-1,4-bis-chlorocarbonic acid ester, hydroquinone-bis-chlorocarbonic acid ester, 4,4'-dihydroxydiphenylene-bis-chlorocarbonic acid ester or 2,2-(4,4' - dihydroxydiphenylene) - propane-bis-chlorocarbonic acid ester, in the presence of inert organic solvents.

When using phosgene or bis-chlorocarbonic acid esters as derivatives of the carbonic acid in producing polycarbonates catalysts also may be advantageous. Such catalysts are for instance tertiary or quaternary organic bases or salts thereof, such as trimethylamine, triethylamine, dimethylaniline, diethylaniline, dimethylcyclohexylamine, and pyridine, or for instance the corresponding hydrochlorides, and tetramethylammoniumhydroxide, triethyloctadecylammoniumchloride, dimethyl - benzyl-phenylammonium-chloride, trimethylcyclohexylammoniumbromide, and N-methylpyridiniumchloride, in amounts from about 0.05 to about 5 percent by weight. These compounds may be added to the reaction mixture before or during the reaction.

Furthermore in some of these cases it is preferable to add surface active agents, such as alkali metal salts of higher fatty acids or of sulphonic acids of higher aliphatic or of aromatic hydrocarbons and polyoxyethylated alcohols and phenols. Greater amounts of the quaternary ammonium bases mentioned above, too, act as such surface active agents.

In the production of polycarbonates according to the various processes it further is advantageous to employ small amounts of reducing agents, for example sodium or

potassium sulphite, sulphite, and dithionite, or free phenol and p-tert.butyl-phenol.

By adding monofunctional compounds which are capable of reacting with phosgene or with the end-groups of the polycarbonates consisting of the chlorocarbonic acid ester group and which terminate the chains, such as the phenols, for instance, phenol, tert. butyl-phenyl-, the cyclo-hexylphenyl-, and 2,2-(4,4'-dihydroxyphenylene-4'-methoxyphenylene)-propane, aniline and methylaniline, it is possible to regulate the molecular weight of the polycarbonates in wide limits.

The working up of the reaction mixture may be effected when operating in the presence of acid-binding agents and organic solvents such as methylene chloride or benzene, in such a manner that the reaction mixture is dissolved cold in dilute sodium hydroxide solution, the organic layer separated, the aqueous layer filtered off and the polycarbonate precipitated from the filtrate by acidification, or that the organic solvent is distilled off from the reaction mixture upon acidification with dilute hydrochloric acid and the polycarbonate filtered off.

The new polycarbonates are soluble in addition to a number of organic solvents such as acetone, tetrahydrofuran, dioxane, dimethyl formamide, mixture of methanol and benzene or ethanol and benzene, further in aqueous alkalies such as sodium or potassium hydroxide or sodium carbonate solution.

The antihalation layers produced from the aforementioned polycarbonates and antihalation dyestuffs known as such are distinguished by sufficient solubility in alkaline silver halide developing solutions even if these are weakly alkaline and contain considerable amounts of salts, furthermore by a good resistance to abrasion and to transfer to emulsions layer disposed in contact with said antihalation layer. The described antihalation layers may be produced on supports of cellulose esters, such as cellulose acetate, cellulose acetobutyrate, nitrocellulose, polyesters of terephthalic acid and glycol, polyvinylchloride and copolymers of vinyl chloride with maleic anhydride or maleic acid esters, polystyrene, and high molecular linear polycarbonates as disclosed for instance in Belgian Patent 532,543. The polycarbonates of the present invention may be applied in admixture with other synthetic or natural resins containing alkali-solubilizing groups, such as copolymers of styrene and acrylic acids, vinylisobutylether and maleic acid, acrylonitrile, vinylbutylether and maleic half esters, celluloseacetatephthalate, polyvinylphthalate. These resins may be combined with the polycarbonates containing alkali-solubilizing groups in the most varied proportions, it is preferred, however, if at least 50 percent of the binding agent consists of said polycarbonates.

The present invention is illustrated by the accompanying drawing representing a cross-section in enlarged scale through a photographic material according to the present invention.

#### Example 1

8 g. of an antihalation dye, such as a dyestuff of the formula:



12 g. of a polycarbonic acid ester from 4,4'-dihydroxy-3,3'-dicarboxyphenyl methane with a K-value of 6

(the K value is defined in "Cellulosechemie," 13, (1932), page 60), are dissolved in the following solvent mixture:

70 parts of ethanol  
20 parts of ethyl acetate  
10 parts of butanol

The solution is applied by the dipping method to the back of an acetyl cellulose film and is dried at approximately 80° C. by air blown thereon. Silver halide emulsions for the production of a multi-layer color photographic material are then applied to the front of the layer support by casting.

The layer dissolves satisfactorily on processing in the photographic baths and does not transfer to the emulsion layer under the conditions prevailing in practice, even with long storage.

The above polycarbonate is produced in the following manner:

Into a solution of 79 parts of 4,4'-dihydroxy-3,3'-dimethyl-5,5'-dicarboxyphenylene-methane, 100 parts of pyridine and 600 parts of methylene chloride, there are introduced with stirring 24.5 parts of phosgene at about 0° C. within 1½ hours. After stirring overnight at room temperature, the solution is treated with 50 parts of water, stirred for 2 minutes and after the addition of 450 parts of 2 N hydrochloric acid stirred for a further 15 minutes. Methylene chloride is subsequently distilled off under vacuum with stirring and the residue is filtered off. The residue remaining after filtration is washed with water until free from chlorine and dried under vacuum at 80° C.

#### Example 2

6 g. of an antihalation dye as for instance a dyestuff of the formula:



according to German application No. A 21525 IVa/57b) (now German Patent 1,008,114).

4 g. of a polyvinyl phthalate according to U.S. patent specification No. 2,131,747, and

55 6 g. of a polycarbonic acid ester with a K value of 10, from 4,4'-dihydroxy-3,3'-dicarboxy-5,5'-dimethyl-diphenyl methane and 2,2-(4,4'-dihydroxy-diphenylene)-propane are dissolved in the following solvent mixture:

60 parts of ethanol  
10 parts of ethyl acetate  
30 parts of isopropanol

The coating is applied to a polycarbonate foil as disclosed in German application No. A 22,482 of Apr. 14, 1955 (now published as No. 1,001,586), and dried. The film is coated with a black-and-white negative emulsion. The properties of the antihalation layer conform to the requirements which have been stated.

The above polycarbonate bonding agent (K=10) is produced as follows:

To a mixture of 17.65 parts of 2,2-(4,4'-dihydroxy-diphenylene)-propane-bis-chlorocarbonic acid ester, 15.15 parts of 4,4'-dihydroxy-3,3'-dicarboxy-5,5'-dimethyl-diphenyl methane and 350 parts of methylene chloride there is added dropwise with stirring at about 0° C.

within 30 minutes a solution of 23.7 parts of pyridine in 40 parts of methylene chloride. After stirring overnight at room temperature, the mixture is acidified with dilute hydrochloric acid and methylene chloride evaporated with stirring in vacuo. After filtration of the residue, the filter residue is washed first with hydrochloric acid and subsequently with water until no further chlorine is detectable in the wash water. The filter residue is dried at 80° C. under vacuo. Further dyestuffs which may be used for the production of the antihalation layers are for instance those disclosed in British specifications 694,681 and 760,739.

*Example 3*

12 g. of an antihalation dye according to U.S. patent specification No. 2,282,890, Example 2;

6 g. of a copolymer of styrene and maleic acid according to U.S. patent specification No. 2,077,789, and

6 g. of a polycarbonate acid ester as referred to in Example 2, are dissolved in the following solvent mixture:

30 parts of ethanol

30 parts of acetone

10 parts of ethyl acetate

30 parts of tetrachloroethane.

The solution is applied to the back of a foil of a polyester of terephthalic acid and glycol having layers of silver halide emulsion on the front.

*Example 4*

A solution of 6 g. of the dyestuff disclosed in Example 1, 4 g. of a copolymer of acrylonitrile, vinylbutylether and maleic acid monoethyl ester (parts by weight: 1:4:5), 6 g. of a polycarbonate of 2,2'-dicarboxy-4,4'-dihydroxy-dicyclohexyl in 90 cc. of ethanol and 10 cc. of butanol is coated on the back of a film of a copolymer of vinyl chloride and maleic acid dimethylester (8:2). A silver halide emulsion layer is then applied to the front of the support. The properties of the antihalation layer conform to the requirements which have been stated.

The polycarbonate is obtained according to the process disclosed in Example 1, replacing the dihydroxy compound of said example by an equimolecular amount of the dihydroxy compound disclosed in the preceding paragraph.

*Example 5*

A solution of 4.7 g. of the dyestuff disclosed in Example 2, 3 g. of a copolymer of an alkali-soluble copolymer of styrene and methacrylic acid according to U.S. specification No. 2,077,789, 5.8 g. of a polycarbonate of 3,6-dihydroxybenzene-dicarboxylic acid-1,2, in 70 g. of isopropanol and 30 g. of ethanol is coated on the back of a nitrocellulose film support and dried. A silver halide emulsion layer is then applied to the front of the support. The antihalation layer meets all requirements.

The polycarbonate is obtained according to the process disclosed in Example 1, replacing the dihydroxy compound of said example by an equimolecular amount of the dihydroxy compound disclosed in the preceding paragraph.

What we claim is:

1. A light-sensitive photographic material comprising a light transmitting support, a photographically light sensitive silver halide gelatin layer coated on one side of said support and an alkali-soluble antihalation layer containing a light absorbing antihalation dyestuff coated on the other side of said support, said antihalation layer containing as a binding agent substantially a major proportion of a high molecular film-forming linear polycarbonate ester of at least one dihydroxy compound selected from the class consisting of aliphatic, cycloaliphatic, araliphatic and aromatic compounds having hydroxy groups selected from the class consisting of alcoholic and phe-

nolic hydroxy groups, at least 30 molar percent of the dihydroxy compound units in the ester also containing from one to two acid groups selected from the class consisting of carboxyl and sulfonic acid groups to render the ester soluble in aqueous alkaline solutions.

2. A light-sensitive photographic material according to claim 1 wherein the ester is the polycarbonate of a di-mono-hydroxy-aryl alkane containing carboxylic acid groups.

3. The combination of claim 1 wherein the support is a film of high molecular weight linear unsubstituted polycarbonate.

4. The combination of claim 1 in which the support is a film of high molecular weight linear unsubstituted polycarbonate, and the alkaline soluble polycarbonate is a carboxylated polycarbonate of a bis-parahydroxy phenyl alkane.

5. The combination of claim 1 in which the dihydroxy compound is bis-(4-hydroxy-3-carboxy phenyl) methane.

6. In combination, a photographically sensitive silver halide emulsion layer on a support, and an antihalo stratum on said support in antihalation relationship with said silver halide emulsion layer, said stratum having a light-absorbing material distributed in a bonding material, at least half of said bonding material being a high molecular weight film-forming linear polycarbonate of at least one dihydroxy compound selected from the class consisting of aliphatic, cycloaliphatic, araliphatic and aromatic compounds having hydroxy groups selected from the class consisting of alcoholic and phenolic hydroxy groups, at least 30 molar percent of the dihydroxy compound units in the polycarbonate also containing from one to two acid groups selected from the class consisting of carboxyl and sulfonic acid groups to render the polycarbonate soluble in aqueous alkaline solutions, any remaining bonding material being an alkali-soluble resin selected from the class consisting of cellulose acetate phthalate, polyvinyl phthalate, and copolymers of styrene with acrylic acids, styrene with maleic acid, vinyl isobutyl ether with maleic acid, and acrylonitrile with vinyl butyl ether and maleic acid half esters.

7. The combination of claim 6 wherein the bonding material is a mixture of a polyvinyl phthalate bonding agent and a polycarbonate of both bis-(4-hydroxy-3-carboxy-5-methyl phenyl) methane and 2,2-bis(parahydroxy phenyl) propane.

8. The combination of claim 6 wherein the bonding material is a mixture of (I) a bonding copolymer of styrene with maleic acid and (II) a polycarbonate of both bis-(4-hydroxy-3-carboxy-5-methyl phenyl) methane and 2,2-bis(parahydroxy phenyl) propane.

9. The combination of claim 6 wherein the bonding material is a mixture of (I) a copolymer of acrylonitrile, vinyl butyl ether, and maleic acid monoethyl ester and (II) a polycarbonate of 2,2'-dicarboxy-4,4'-dihydroxy-dicyclohexyl.

10. The combination of claim 6 wherein the bonding material is a mixture of (I) a bonding copolymer of styrene with methacrylic acid and (II) a polycarbonate of 3,6-dihydroxybenzene-dicarboxylic acid-1,2.

References Cited in the file of this patent

UNITED STATES PATENTS

|    |           |                |               |
|----|-----------|----------------|---------------|
| 65 | 1,884,035 | Malm           | Oct. 25, 1932 |
|    | 2,455,653 | Bralley et al. | Dec. 7, 1948  |
|    | 2,461,485 | Thompson       | Feb. 8, 1949  |
|    | 2,462,527 | McQueen        | Feb. 22, 1949 |
|    | 2,536,989 | Glahn et al.   | Jan. 2, 1951  |

70

FOREIGN PATENTS

|         |         |               |
|---------|---------|---------------|
| 372,933 | Germany | Apr. 23, 1953 |
| 532,543 | Belgium | Oct. 30, 1954 |